

[54] **TANNING COMPOSITION AND PROCESS**

[76] Inventor: **Reid S. Larsen**, 762 S. 850 East, Bountiful, Utah 84010

[22] Filed: **Jan. 11, 1973**

[21] Appl. No.: **322,815**

[52] U.S. Cl. .... **8/94.19 R**, **8/94.18**

[51] Int. Cl. .... **C14c 3/02**, **C14c 3/04**

[58] Field of Search..... **8/94.18**, **94.19 R**, **94.22**

[56] **References Cited****UNITED STATES PATENTS**

|           |         |               |       |           |
|-----------|---------|---------------|-------|-----------|
| 110,562   | 12/1870 | Fuller et al. | ..... | 8/94.22   |
| 118,746   | 9/1871  | Rock          | ..... | 8/94.18   |
| 1,567,644 | 8/1921  | Hell          | ..... | 8/94.19 R |
| 3,512,918 | 5/1970  | Endres et al. | ..... | 8/94.19 R |

**OTHER PUBLICATIONS**

Chakrovorty et al., "Uncommon Inorganic Tannages"

Vol. XLII No. 1 Jan. 1958 pp. 2-10.

Pavis; Manufacture of Leather 1885 London pp. 52-53 Journal of Society of Leather Trades Chemist.

*Primary Examiner*—Benjamin R. Padgett

*Assistant Examiner*—B. Hunt

*Attorney, Agent, or Firm*—H. Ross Workman

[57] **ABSTRACT**

A tanning composition and process, the composition including a salt of carbonic acid, arsenic trioxide, a polar solvent and a liquid organic cleanser all mixed with sufficient ground asbestos to give a spreadable texture to the composition. The process includes placing the described tanning composition on the flesh side of the skin and allowing the composition to remain until dry or crystallized whereupon the dry composition is removed by abrading.

**5 Claims, No Drawings**

**TANNING COMPOSITION AND PROCESS****BACKGROUND****1. Field of the Invention**

The invention relates to the tanning of hides and skins and more particularly to a novel tanning composition of matter which is both easy to use and effective in tanning hides and a process for using same.

**2. The Prior Art**

Numerous tanning compositions are known in the art. However, the texture of the various compositions often makes the composition extremely difficult to work with. For example, powders are uniformly applied only with great difficulty and uneven application tends to reduce the quality of the tan.

Liquid tanning compositions are also used with difficulty. Many liquid tanning compositions are often very unstable and vital components rapidly precipitate making a suitable uniform tan difficult if not impossible. Frequently, liquid tanning compositions must be freshly prepared and used with costly and complicated machinery to obtain an effective tan. Machine tanning often undesirably adversely affects the quality of fur-bearing pelts and is most undesirable when the tanned pelt is to be taxidermically restored.

In the treatment of hides and pelts, it is desirable to have a tanning composition which is easily applied, effects an adequate tan and will not injure the hide or pelt even though the composition is left on the pelt for an extended period of time. This present invention uniquely accommodates these desirable advantages.

**BRIEF DESCRIPTION AND OBJECTS OF THE INVENTION**

The present invention, including composition of matter and process, provides a tanning composition containing ground asbestos which prevents premature separation of solids from solution and at the same time gives the tanning composition a texture which accommodates facile handling. The composition and method allow pelts to be tanned without injury even though the tanning composition remains on the pelt for an extended period of time.

It is, therefore, a primary object of the present invention to provide a novel tanning composition.

It is another primary object of the present invention to provide an improved method of tanning hides and pelts without injury thereto.

These and other objects and features of the present invention will become more fully apparent from the following description and appended claims.

**DETAILED DESCRIPTION OF THE PREFERRED EMBODIMENTS****THE COMPOSITION**

The presently preferred tanning composition is a combination of arsenic trioxide and salt of carbonic acid in a polar solvent such as methanol. This portion of the composition is effective to tan most pelts but it is often desirable to simultaneously cleanse the flesh side of the pelt without damage thereto. Accordingly, a quantity of kerosene is added to facilitate cleansing fatty material from the pelt in concert with the tanning process. Any suitable organic cleaner that will not interfere with the tanning process could be used.

It has been found that the solids in this preparation can be maintained essentially uniformly disbursed by

mixing sufficient ground asbestos to give the composition a viscous, paste-like consistency. The asbestos is resistant to degradation by the chemical components of the composition and lends consistency to the composition without significantly adversely affecting the tanning process.

Preferably, a suitable anti-bacterial agent such as sodium pentachlorophenol is used to minimize the bacterial degradation of the pelt. Also, it is often desirable to use a suitable conventional coloring agent to finish the tanned pelt.

The following examples illustrate the invention:

**EXAMPLE 1**

15 A composition for tanning pelts was prepared having the formulation shown in Table A.

**TABLE A**

|    | Ingredient               | Amount    |
|----|--------------------------|-----------|
| 20 | Sodium bicarbonate       | 200 lbs   |
|    | Arsenic trioxide         | .25 lbs   |
|    | Sodium pentachlorophenol | .375 lbs  |
|    | Ground asbestos          | 1 lb      |
|    | Methanol                 | 6 quarts  |
| 25 | Kerosene                 | 44 quarts |

The composition was prepared by thoroughly mixing the sodium bicarbonate, ground asbestos and arsenic trioxide. In a separate container, the sodium pentachlorophenol was dissolved in methanol at room temperature. The kerosene and methanol solution of sodium pentachlorophenol were then poured over the dry mix and stirred continuously until thoroughly blended. The composition was easily applied by spreading upon a fresh pelt and the pelt was tanned when exposed to the composition for 24 hours. No injury to the pelt was evident even when the pelt was exposed to the composition for 2 weeks duration.

**EXAMPLE 2**

40 A composition was formed as described in Example 1 except that the amount of sodium bicarbonate was reduced to 170 pounds. The pelt was adequately tanned when used as described above.

**EXAMPLE 3**

45 A composition was prepared as in Example 1 except that the sodium bicarbonate was increased to 230 pounds. In this example, the tan of the pelt was not as advanced after 24 hours as was evident in the Example 1 composition.

**EXAMPLE 4**

50 A composition was prepared as in Example 1 except that sodium carbonate was substituted for sodium bicarbonate. The tanning ability of the composition was somewhat adversely affected.

**EXAMPLE 5**

60 A composition was prepared as in Example 1 except that potassium bicarbonate was substituted for sodium bicarbonate. The tanning ability of the composition was somewhat adversely affected.

**EXAMPLE 6**

A series of compositions having the proportions set forth in Example 1 were prepared except that the

amount of ground asbestos was incrementally increased in 0.25 pound amounts in the range of from 0.75 pounds to 1.5 pounds. It was found that where the ground asbestos was reduced over that proportion of Example 1, the product was not sufficiently viscous to accommodate facile spreadability. It was found that as the amount of ground asbestos incrementally increased, the viscosity correspondingly increased. Even when the composition was very thick, the tanning ability of the composition did not appear to be adversely affected. 10

#### EXAMPLE 7

It was found that the amount of kerosene set forth in Table 1 could be varied in amounts from at least as low as 30 quarts to at least as high as 60 quarts without adversely affecting the tanning ability of the formulation. It was observed, however, that if the amount of kerosene was altered substantially, the amount of ground asbestos required corresponding adjustment to effect 20 desirable viscosity.

#### THE PROCESS

The tanning composition set forth above is placed on the flesh side of a pelt by spreading the composition in a thin layer over the pelt. Preferably, the thickness of the composition is less than one-quarter inch. The composition is allowed to remain on the pelt preferably until the composition has dried to crystals. Normally, drying will take place in 24 to 48 hours. It has been found, however, that tanning may be complete before the composition is completely dry. 25

The crystallized composition is preferably removed from the skin by abrading with an abrasive such as sandpaper. As the composition is removed, the pelt is 35 tanned and completely freed of fatty material. Moreover, the abrasive imparts a highly desirable softness into the pelt.

When the tanning composition has been removed, it is sometimes desirable to treat the pelt with conventional oil or the like which further softens the pelt and may preserve the pelt from drying. Also, if desired, the pelt can be colored at this point in the process. 40

Where coloration of the pelt is desirable, conventional coloring material may be dissolved with the sodium pentachlorophenol in methanol as described in Example 1. The color will then be imparted to the pelt upon application of the tanning composition. 5

The invention may be embodied in other specific forms without departing from its spirit or essential characteristics. The described embodiments are to be considered in all respects only as illustrative and not restrictive and the scope of the invention is, therefore, indicated by the appended claims rather than by the foregoing description. All changes which come within the meaning and range of equivalency of the claims are to be embraced within their scope.

15 What is claimed and desired to be secured by United States letters Patent is:

1. A tanning composition comprising arsenic trioxide; a polar solvent; a liquid organic cleanser and ground asbestos together with a salt of carbonic acid selected from the group consisting of sodium carbonate, sodium bicarbonate, potassium carbonate and potassium bicarbonate.

2. A tanning composition as defined in claim 1 further comprising an anti-bacterial agent.

3. A tanning composition as defined in claim 2 wherein said anti-bacterial agent is sodium pentachlorophenol.

4. A process for tanning a skin comprising: placing on the flesh side of the skin a thin layer of tanning composition comprising arsenic trioxide, a polar solvent, a liquid organic cleanser and ground asbestos and a salt of carbonic acid selected from the group consisting of sodium carbonate, sodium bicarbonate, potassium carbonate and potassium bicarbonate; allowing the tanning composition to remain upon the skin until dry; and removing the dried composition by rubbing with an abrasive.

40 5. A method of tanning a skin as defined in claim 4 further comprising treating the skin with oil by rubbing oil on the tanned surface.

\* \* \* \* \*